

3,705,809

## SILVER HALIDE SUPERSENSITIZED PHOTOGRAPHIC EMULSION

Yoshiyuki Nakazawa, Yashuharu Nakamura, Haruo Takei, Akira Sato, and Tadashi Ikeda, Kanagawa, Japan, assignors to Fuji Photo Film Co., Ltd., Kanagawa, Japan  
No Drawing. Filed Oct. 20, 1970, Ser. No. 82,537  
Claims priority, application Japan, Sept. 26, 1969,

44/76,684

Int. Cl. G03c 1/14

U.S. Cl. 96—124

10 Claims

### ABSTRACT OF THE DISCLOSURE

A silver halide photographic emulsion containing a combination of sensitizing dyes of the formulae:



and



Specific compounds are disclosed hereinafter.

### BACKGROUND OF THE INVENTION

#### Field of the invention

This invention relates to the spectral sensitization of silver halide photographic emulsions and, more particularly, to silver halide photographic emulsions which have been super-sensitized by a combination of sensitizers of two different types. In particular, it is concerned with silver halide photographic emulsions having high red sensitivities and spectral sensitization maxima within the region between 625m $\mu$  and 665 m $\mu$ .  
45

### DESCRIPTION OF THE PRIOR ART

It is well known in the art of silver halide photographic emulsions that the range of the sensitive wave length of a silver halide emulsion is extended and the silver halide emulsion is spectrally sensitized by the addition thereto of a sensitizing dye.

Although sensitization of photo-sensitive materials in a desired spectral range of wave length may usually be attained by the use of a single sensitizing dye, in many cases there are used combinations of two or more sensitizers. Usually, the degree of spectral sensitization brought about by the use of a combination of two or more sensitizers is between those values achieved by the separate use of each sensititizer or even lower than that intermediate value. However, in certain cases, there are obtained remarkably higher degrees of spectral sensitization than those obtained by the sole use of one of the sensitizers. This phenomenon is usually referred to as "super sensitization." Even then, the sensitized range of wave length occasionally lies in the middle of those values obtained by the use of the individual sensitizers alone.

In the manufacture of silver halide photographic emulsions, a combination of two or more sensitizers of different types is often used for either sensitization in a desired spectral wave length region as a means for obtaining a

higher spectral sensitivity than that obtained by the individual use of the sensitizers or controlling the spectrally sensitized wave length region of the emulsion to a certain wave length region.

- 5 It has been a significant problem in spectral sensitization techniques to find a combination of sensitizers in the relationship of super sensitization such that there is obtain a higher spectral sensitivity by the use of a combination of sensitizers than that obtained by the use of the 10 individual sensitizers, or that the sensitized wave length region is controlled so as to meet the requirements for the photo-sensitive material.

It is an object of the present invention to provide a silver halide photographic emulsion having a high red 15 sensitivity in the spectrally sensitized wave length region of from 625 m $\mu$  to 665 m $\mu$  by the use of a combination of sensitizers of two different types. This spectral wave length region is one which is ordinarily adopted in monochromatic photo-sensitive materials and in red-sensitive 20 layers in color photo-sensitive materials.

### SUMMARY OF THE INVENTION

The above object of the present invention has been attained by adding to a silver halide photographic emulsion 25 a combination of a sensitizing dye represented by the following Formula I and a sensitizing dye represented by the following Formula II:



### DESCRIPTION OF THE PREFERRED EMBODIMENTS

In the above Formula I, Z<sub>1</sub> and Z<sub>2</sub>, which may be the same or different, each represents sulfur or selenium atoms; R<sub>1</sub> represents a hydrogen atom or a lower alkyl group such as methyl or ethyl; W<sub>1</sub> represents a hydrogen atom; W<sub>2</sub> represents a hydrogen atom or a halogen atom such as chlorine or bromine, or a lower alkyl group such as methyl or ethyl, or an alkoxy group such as methoxy or ethoxy group, or an aryl group such as phenyl, or a hydroxyl group; or W<sub>1</sub> and W<sub>2</sub> in combination each represents an atomic group necessary to complete a benzene ring; R<sub>2</sub> and R<sub>3</sub> each represents  $\gamma$ -sulfopropyl,  $\gamma$ -sulfonylpropyl,  $\delta$ -sulfonylbutyl or vinylmethyl groups; R<sub>4</sub> represents an ethyl group or an aryl group such as phenyl; X<sub>1</sub> represents an acid anion group usually employed in dyes of this type such as chloride, bromide, iodide, perchlorate, thiocyanate, p-toluenesulfonate, benzene sulfonate, methyl sulfate, ethyl sulfate, and the like; and n represents 0 or 1. In the case of an intramolecular salt, n is 0.

In the above Formula II, Z<sub>3</sub> and Z<sub>4</sub>, which may be the same or different, each represents sulfur or selenium atoms; W<sub>3</sub> and W<sub>4</sub>, which may be the same or different, each represents hydrogen or halogen atoms, or methyl, methoxy, an aryl group such as phenyl, or a hydroxyl group; R<sub>7</sub> represents a methyl or ethyl group, wherein at least one of W<sub>3</sub> and W<sub>4</sub> is other than a hydrogen atom 65 when R<sub>7</sub> is a methyl group; R<sub>5</sub> and R<sub>6</sub>, which may be the same or different, each represents a lower alkyl group such as methyl or ethyl, a substituted alkyl group such as

$\gamma$ -sulfopropyl,  $\gamma$ -sulfobutyl,  $\delta$ -sulfobutyl,  $\beta$ -hydroxyethyl,  $\beta$ -carboxyethyl or  $\gamma$ -carboxypropyl, or an allyl group such as vinyl methyl;  $X_2$  represents an anion such as described in  $X_1$  of the Formula I, and  $n$  represents 0 to 1. In the case of an intramolecular salt,  $n$  is 0.

The present inventors have found that a high red sensitivity is obtained by the use, in combination, of sensitizing dyes (I) and (II) to effect an interactive remarkable super sensitization. The sensitizing dyes according to the present invention may be used in combination with other sensitizers having different spectral sensitization ranges, e.g., a sensitizer for enhancing green sensitivity such as pseudo-cyanin.

Specific embodiments of the sensitizing dyes used in the present invention are represented by the following formulae, but the present invention should not be limited to these merely illustrative compounds:





The sensitizing dyes (I) and (II) may be synthesized by known processes. For instance, synthesis may be attained without difficulty by referring to U.S. Pat. Nos. 2,503,776 and 2,647,051.

The synthesis of sensitizing dye I-C, as listed above, is illustrated hereinafter as a representative example of a typical synthesis.

A mixture of 1.5 g. of 5-phenyl-3-ethyl-2-thiopropionylmethylene-benzothiazoline and 1.5 g. of methyl paratoluenesulfonate is heated at 110° C. for 2 hours and, after cooling, the reaction mixture is washed with ethyl ether. 1.5 g. of anhydro-5-carboxy-2-methyl-3-( $\gamma$ -sulfopropyl)-benzothiazolium hydroxide, dissolved in 160 ml. of ethanol, is then added to the reaction product, refluxed for 3 hours in the presence of 5 ml. of triethylamine and freed from solvent by distillation. The residue is crystallized by treatment with ethyl ether. The crystals are recovered by filtration, thoroughly washed with acetone and recrystallized from a methanol-chloroform mixture

75 to obtain 1.1 g. of a dye having a M.P. of 287° C. and a

$\lambda_{\text{max.}}^{\text{MeOH}}$

5

of 559 nm.

The other sensitizing dyes of the present invention may be synthesized by methods similar to that described above.

10 The spectral sensitization process of the present invention is effective for the spectral sensitization of gelatino silver halide emulsions. In the process, emulsions containing a synthetic or natural hydrophilic resinous material other than gelatin, such as agar agar, water-soluble cellulose derivatives, colloidion or polyvinyl alcohol, may also be sufficiently sensitized.

The photographic emulsion suitable used in the present invention includes silver iodobromide, silver chlorobromide and like mixed silver halide emulsions.

20 The spectrally sensitized photographic emulsion of the present invention may be prepared by incorporating the sensitizing dyes (I) and (II) in a photographic emulsion in a conventional manner. In practice, it is usual to add a solution of the dyes to an emulsion in a suitable solvent, such as methanol or ethanol. The molar ratio of sensitizing dye (I) to dye (II) may be varied in a wide range of from 9:1 to 1:9, according to the desired effects.

Generally, from 0.009 to 0.14 mole of each of dyes (I) and (II) may be added to each 1 kg. of emulsion.

30 The photographic emulsion of the present invention may also be subjected to a hyper-sensitization by known processes.

In the preparation of the photographic emulsion of the present invention there may also be incorporated in the emulsion conventional additives such as, e.g., a sensitizer, 35 a stabilizer, a toner, a hardener, a surface active agent, an anti-fogging agent, a plasticizer, a developing promoter, a color developer and an optical whitening agent.

The photographic emulsion of the present invention 40 may be applied to a suitable support such as, e.g., sheet glass, a film of a cellulose derivative, a film of a synthetic resin or baryta paper in a conventional manner.

The present invention will now be illustrated in more detail by the following examples, which are not intended 45 to be limiting in nature.

## EXAMPLES

To separate portions of a silver iodobromide emulsion 50 in which the molar ratio of AgI to AgBr was 7:93, and where the emulsion contained about 25.4 g. of silver per 1 kg. of emulsion, there was added a sensitizing dye (I) alone, a sensitizing dye (II) alone or a combination of (I) and (II) to form sensitized silver halide emulsions. 55 The emulsions were separately applied to triacetylcellulose film bases and, after drying, exposed to a light of day light color corresponding to a color temperature of 5,400° K. through a Fuji filter No. 7 (trademark; (a red filter transmitting light having a wave length of 580 nm or more) supplied by Fuji Photo Film Co., Ltd., and then developed using a developing solution of the formulation as indicated in Table 1.

TABLE 1

|                        | G.  |
|------------------------|-----|
| 65 Metol -----         | 2   |
| Sodium sulfite -----   | 100 |
| Hydroquinone -----     | 5   |
| Borax -----            | 2   |
| Water to make 1 liter. |     |

In the following Table 2 are shown the spectral sensitivity and sensitization maxima obtained by using the sensitizing dye (I) alone, as described above. In the following Table 3 are indicated those obtained by using the sensitizer dye (II) alone, as described above. In Table 4

are indicated those obtained by combinations of representative sensitizing dyes (I) and (II).

TABLE 2

| Dye number | Amount of dye added (10 <sup>-5</sup> mol/kg. emulsion) | Emulsion | Sensitization maxima (nm.) | Red sensitivities |
|------------|---------------------------------------------------------|----------|----------------------------|-------------------|
| A          | 8                                                       | AgBr/I   | 643                        | 230               |
| B          | 8                                                       | AgBr/I   | 650                        | 370               |
| C          | 8                                                       | AgBr/I   | 625                        | 100               |
| D          | 6                                                       | AgBr/I   | 652                        | 250               |
| E          | 8                                                       | AgBr/I   | 647                        | 300               |
| F          | 4                                                       | AgBr/I   | 643                        | 150               |
| G          | 8                                                       | AgBr/I   | 650                        | 250               |
| H          | 6                                                       | AgBr/I   | 628                        | 130               |
| I          | 4                                                       | AgBr/I   | 650                        | 260               |
| J          | 8                                                       | AgBr/I   | 654                        | 82                |
| K          | 8                                                       | AgBr/I   | 656                        | 160               |
| L          | 8                                                       | AgBr/I   | 645                        | 72                |

The red sensitivity is indicated as the specific sensitivity regarding the red sensitivity of sensitizing dye C upon exposure through a Fuji filter No. 7 (red filter) as 100.

TABLE 3

| Dye number | Amount of dye added (10 <sup>-5</sup> mol/kg. emulsion) | Emulsion | Sensitization maxima (nm.) | Red sensitivities |
|------------|---------------------------------------------------------|----------|----------------------------|-------------------|
| 1          | 8                                                       | AgBr/I   | 640-650                    | 128               |
| 2          | 8                                                       | AgBr/I   | 662                        | 250               |
| 3          | 8                                                       | AgBr/I   | 660                        | 250               |
| 4          | 6                                                       | AgBr/I   | 635                        | 145               |
| 5          | 8                                                       | AgBr/I   | 632                        | 230               |
| 6          | 6                                                       | AgBr/I   | 680                        | 160               |
| 7          | 8                                                       | AgBr/I   | 680                        | 270               |
| 8          | 6                                                       | AgBr/I   | 590-600                    | 44                |
| 9          | 8                                                       | AgBr/I   | 638                        | 130               |
| 10         | 8                                                       | AgBr/I   | 590-610                    | 74                |
| 11         | 6                                                       | AgBr/I   | 658                        | 250               |
| 12         | 8                                                       | AgBr/I   | 660                        | 150               |

The red sensitivity is indicated as the specific sensitivity regarding the red sensitivity of sensitizing dye C upon exposure through a Fuji filter No. 7 (red filter) as 100.

TABLE 4

| Example No. | Dye Number | Amount of dye added (10 <sup>-5</sup> mol/kg. emulsion) | Emulsion | Sensitization maxima (nm.) $\mu$ | Red sensitivities |
|-------------|------------|---------------------------------------------------------|----------|----------------------------------|-------------------|
|             | A          | 8                                                       | AgBr/I   | 643                              | 230               |
|             | 2          | 8                                                       | AgBr/I   | 662                              | 250               |
|             | 5          | 8                                                       | AgBr/I   | 632                              | 230               |
| 1           | { A+2      | 4+3                                                     | AgBr/I   | 656                              | 370               |
|             | A+5        | 6+2                                                     | AgBr/I   | 643                              | 370               |
|             | B          | 8                                                       | AgBr/I   | 650                              | 370               |
|             | 9          | 8                                                       | AgBr/I   | 638                              | 130               |
| 2           | B+9        | 6+2                                                     | AgBr/I   | 648                              | 470               |
|             | C          | 8                                                       | AgBr/I   | 625                              | 100               |
|             | J          | 8                                                       | AgBr/I   | 654                              | 82                |
|             | 3          | 8                                                       | AgBr/I   | 660                              | 250               |
| 3           | { C+3      | 2+6                                                     | AgBr/I   | 655                              | 310               |
|             | J+3        | 2+6                                                     | AgBr/I   | 660                              | 300               |
|             | D          | 6                                                       | AgBr/I   | 652                              | 250               |
|             | 2          | 8                                                       | AgBr/I   | 662                              | 250               |
| 4           | D+2        | 4+3                                                     | AgBr/I   | 658                              | 340               |
|             | E          | 8                                                       | AgBr/I   | 647                              | 390               |
|             | 4          | 6                                                       | AgBr/I   | 635                              | 145               |
|             | 7          | 8                                                       | AgBr/I   | 660                              | 270               |
| 5           | { E+4      | 6+2                                                     | AgBr/I   | 645                              | 470               |
|             | E+7        | 6+2                                                     | AgBr/I   | 650                              | 500               |
|             | F          | 4                                                       | AgBr/I   | 643                              | 150               |
|             | 1          | 8                                                       | AgBr/I   | 640-650                          | 128               |
|             | 6          | 6                                                       | AgBr/I   | 680                              | 160               |
| 6           | { F+1      | 3+3                                                     | AgBr/I   | 648                              | 330               |
|             | F+6        | 6+2                                                     | AgBr/I   | 664                              | 360               |
|             | G          | 8                                                       | AgBr/I   | 650                              | 250               |
|             | 3          | 8                                                       | AgBr/I   | 660                              | 250               |
|             | 8          | 6                                                       | AgBr/I   | 590-600                          | 44                |
| 77          | { G+3      | 2+6                                                     | AgBr/I   | 660                              | 340               |
|             | G+8        | 7+1                                                     | AgBr/I   | 660                              | 320               |
|             | G+12       | 6+2                                                     | AgBr/I   | 658                              | 310               |
|             | H          | 6                                                       | AgBr/I   | 628                              | 130               |
|             | 10         | 8                                                       | AgBr/I   | 590-610                          | 74                |
| 8           | H+10       | 6+2                                                     | AgBr/I   | 628                              | 220               |
|             | I          | 4                                                       | AgBr/I   | 650                              | 260               |
|             | II         | 6                                                       | AgBr/I   | 658                              | 250               |
| 9           | I+11       | 2+6                                                     | AgBr/I   | 655                              | 320               |
|             | 3          | 8                                                       | AgBr/I   | 660                              | 250               |
|             | K          | 8                                                       | AgBr/I   | 656                              | 160               |
|             | L          | 8                                                       | AgBr/I   | 645                              | 72                |
| 10          | { 3+K      | 6+2                                                     | AgBr/I   | 660                              | 300               |
|             | 3+L        | 6+2                                                     | AgBr/I   | 660                              | 290               |

The red sensitivity is indicated as the specific or relative sensitivity calculated by regarding the specific or 75

relative sensitivity of sensitizing dye C upon exposure through a Fuji filter No. 7 (red filter) as 100.

As is evident from Table 4, a remarkably higher enhancement in red sensitivity is obtained by the use of a combination of the sensitizing dyes (I) and (II) than that obtained by the use of sensitizing dyes (I) or (II) alone.

What is claimed is:

1. A silver halide photographic emulsion containing a combination of at least one sensitizing dye of the Formula I and at least one sensitizing dye of the Formula II:



wherein, in Formula I,  $Z_1$  and  $Z_2$ , which may be the same or different, each represents a sulfur or selenium atom;  $R_1$  represents a hydrogen atom or a lower alkyl group;  $W_1$  represents a hydrogen atom, a halogen atom, a lower alkyl group, an alkoxy group, an aryl group or a hydroxyl group, or in combination  $W_1$  and  $W_2$  represent atomic groups necessary to complete a benzene ring;  $R_2$  and  $R_3$  each represent an ethyl, n-propyl,  $\gamma$ -sulfopropyl,  $\gamma$ -sulfobutyl,  $\delta$ -sulfobutyl or vinylmethyl group;  $R_4$  represents an ethyl or aryl group;  $X$  represents an anion, and  $n$  represents 0 or 1, where, in the case of an intramolecular salt,  $n=0$ ; and, in Formula II,  $Z_3$  and  $Z_4$ , which may be the same or different, each represent a sulfur or selenium atom;  $W_3$  and  $W_4$ , which may be the same or different, each represents a hydrogen atom, halogen atom, methyl, methoxy, aryl or hydroxyl group;  $R_7$  represents a methyl or ethyl group, wherein at least one of  $W_3$  and  $W_4$  is other than hydrogen when  $R_7$  is a methyl group;  $R_5$  and  $R_6$  represent lower alkyl, a substituted lower alkyl from the group consisting of sulfoalkyl, carboxyalkyl or hydroxyalkyl, or an allyl group;  $X$  represents an anion; and  $n$  represents 0 or 1 and, in the case of an intramolecular salt,  $n=0$ .

2. A silver halide photographic emulsion as claimed in claim 1 wherein the lower alkyl group in  $R_1$ ,  $R_5$ ,  $R_6$  and  $W_2$  is an alkyl group having from 1 to 4 carbon atoms.

3. A silver halide photographic emulsion containing a combination of at least one sensitizing dye selected from the group consisting of





and at least one sensitizing dye selected from the group consisting of,



11



and



4. The silver halide photographic emulsion as claimed in claim 1 wherein the molar ratio of the sensitizing dye of Formula I to the sensitizing dye of Formula II is within the range of from 1:9 to 9:1.

5. A photographic light-sensitive element comprising a support having thereon at least one layer containing the silver halide emulsion as claimed in claim 1.

6. The silver halide photographic emulsion as claimed in claim 4 having a high red sensitivity in the spectrally sensitized wavelength region of from 625 m $\mu$  to 665 m $\mu$  wherein from 0.009 to 0.14 mol of each of the dyes of Formula I and II is added to 1 kg. of emulsion.

7. The photographic light-sensitive element as claimed in claim 5 wherein the molar ratio of the sensitizing dye

12

of Formula I to the sensitizing dye of Formula II is within the range of from 1:9 to 9:1.

8. The photographic light-sensitive element as claimed in claim 5 having a high red sensitivity in the spectrally sensitized wavelength region of from 625 m $\mu$  to 665 m $\mu$  wherein from 0.009 to 0.14 mol of each of the dyes of Formula I and II is added to 1 kg. of emulsion.

9. The silver halide photographic emulsion as claimed in claim 6 wherein Z<sub>1</sub> and Z<sub>2</sub> are both sulfur or one of Z<sub>1</sub> and Z<sub>2</sub> is sulfur and the other is selenium, and wherein Z<sub>3</sub> and Z<sub>4</sub> are both sulfur or wherein Z<sub>3</sub> and Z<sub>4</sub> are both selenium.

10. A photographic light-sensitive element as claimed in claim 9 wherein Z<sub>1</sub> and Z<sub>2</sub> are both sulfur or one of Z<sub>1</sub> and Z<sub>2</sub> is sulfur and the other is selenium, and wherein Z<sub>3</sub> and Z<sub>4</sub> are both sulfur or wherein Z<sub>3</sub> and Z<sub>4</sub> are both selenium.

#### References Cited

#### UNITED STATES PATENTS

|           |        |                 |       |        |
|-----------|--------|-----------------|-------|--------|
| 2,647,050 | 7/1953 | Firestone       | ----- | 96—137 |
| 2,647,051 | 7/1953 | Vinton et al.   | ----- | 96—137 |
| 3,527,641 | 9/1970 | Nakazawa et al. | ----- | 96—124 |
| 3,573,920 | 4/1971 | Hiller          | ----- | 96—124 |

J. TRAVIS BROWN, Primary Examiner

U.S. Cl. X.R.

96—137, 142